# EUROPEAN PATENT SPECIFICATION

(11) **EP 2 091 733 B1**
(45) Date of publication and mention of the grant of the patent: **29.05.2013**
(21) Application number: 07817073.5
(22) Date of filing: 12.10.2007
(51) Int. Cl.: B32B 33/00, B32B 27/28, B05D 7/24, B05D 1/36, B05D 3/06, B05D 5/06, C08J 7/00, G06F 3/02, H01H 13/14, H04M 1/23, B05D 7/00

(54) **MULTI-LAYER COATED PRODUCT AND PREPARATION METHOD THEREOF**
MEHRLAGIGES BESCHICHTETES PRODUKT UND HERSTELLUNGSVERFAHREN DAFÜR
PRODUIT ENDUIT MULTICOUCHES ET PROCÉDÉ DE PRÉPARATION DUDIT PRODUIT

(30) Priority: 08.12.2006 CN 200610153118
(43) Date of publication of application: 26.08.2009
(73) Proprietor: Byd Company Limited, Shenzhen, Guangdong 518119 (CN)
(72) Inventor: LIU, Meng, Guangdong 518119 (CN); LI, Zhixin, Guangdong 518119 (CN)
(74) Representative: HOFFMANN EITLE
(86) International application number: PCT/CN2007/070882
(87) International publication number: WO 2008/067741

(56) References cited:
- EP-A1- 1 123 791
- EP-A2- 1 320 115
- CN-A- 1 208 883
- CN-Y- 2 179 984
- US-A- 5 894 039
- US-A- 5 894 039

## Description

### Field of the Invention

The present invention relates to a multi-layer coated product and a preparation method thereof.

### Background of the Invention

Presently, with the development of electronic products, increasingly more attention is paid to keys or keyboards which are functional components of the electronic products. The keys or keyboards of electronic products such as a mobile telephone, an electronic dictionary, or a personal digital assistant (PDA), are usually prepared by coating plastics as a substrate with two layers of coating (i.e., an undercoat and a topcoat), to obtain multi-layer coated products; and then, removing the topcoat on the backlight part of the key or the keyboard (i.e., the part with letter or pattern), to expose the undercoat on the part, so that the undercoat shows backlight color, while the topcoat shows the shell color.

European patent application EP 1 320 115 A2 discloses a keypad and method of separating a cross-linked cured resin layer thereof. The United States patent US 5,894,039 is concerned with a manufacturing method of a water-cover type transparent keyboard. The use of a polyvinyl chloride -acetate resin in a primer composition is known from European patent application EP1 123 791 A1.

The topcoat on the backlight part is usually removed by laser engraving, at an appropriate laser intensity to ensure that the topcoat is completely removed but the undercoat is not affected. Accordingly, it takes a long testing time to determine the appropriate laser intensity. Furthermore, since the topcoat on different parts of the same key or keyboard may have a different thickness, above requirement may not be met with the same laser intensity, and as a result, the production efficiency will be lowered.

Moreover, in order to prevent the undercoat from being affected during the laser engraving, the laser intensity used in the laser engraving is usually slightly lower than those required for completely removing the topcoat, such that residual topcoat may remains on the backlight part after the laser engraving, and has to be removed by scrubbing with alcohol. In order to prevent the undercoat and the topcoat on other parts from being scrubbed off by alcohol, the undercoat and topcoat both have the alcohol resistance; therefore, it takes a long time to scrub off the residual topcoat on the backlight part with alcohol, and as a result, the production efficiency is lowered.

As described above, the multi-layer coated products of the prior art have the drawback of low production efficiency.

### Summary of the Invention

The object of the present invention is to provide a multi-layer coated product featured with high production efficiency and the preparation method thereof, so as to overcome the drawback of low production efficiency of the prior art multi-layer coated products.

The present invention provides a multi-layer coated product, comprising:
a substrate, and
a multi-layer coating including an undercoat and a topcoat which are formed on the substrate in sequence, have alcohol resistance, and are in a different color from each other, wherein the multi-layer coating further includes an intermediate coat having no alcohol resistance between the undercoat and the topcoat.

The present invention also provides a preparation method for the multi-layer coated product, including the step of forming an undercoat and a topcoat which have alcohol resistance and are in a different color from each other on a substrate in sequence, wherein it further includes the step of forming an intermediate coat having no alcohol resistance between the undercoat and the topcoat.

The multi-layer coated product provided by the present invention comprises a substrate and a multi-layer coating comprising an undercoat, an intermediate coat, and a topcoat formed on the substrate in sequence, wherein the undercoat and the topcoat both have the alcohol resistance, while the intermediate coat has no alcohol resistance. When the intermediate coat and topcoat on the backlight part are removed by the laser engraving, it is sufficient that the laser intensity is controlled to be higher than the laser intensity required for completely removing the topcoat and lower than the laser intensity that affects the undercoat. Even if the laser intensity is lower than the laser intensity required for completely removing the intermediate coat and the topcoat, the residual intermediate coat having no alcohol resistance on the backlight part can be removed easily with alcohol or alcoholic solution, while the topcoat and undercoat having alcohol resistance will not be scrubbed off by the alcohol or alcoholic solution. Therefore, the time required for determining the laser intensity and scrubbing can be shortened, and thereby the production efficiency of said multi-layer coated product can be improved.

### Detailed Description of the Embodiments

The multi-layer coated product provided by the present invention comprises:
a substrate, and
a multi-layer coating including an undercoat and a topcoat which are formed on the substrate in sequence, have alcohol resistance, and are in a different color from each other, wherein the multi-layer coating further includes an intermediate coat having no alcohol resistance between the undercoat and the topcoat.

Said undercoat and topcoat can be the same with the undercoat and topcoat on the keys or keyboards of electronic products in the prior art.

Said undercoat, topcoat, and intermediate coat can each independently have a thickness of 3 to 15 µm, preferably 5 to 9 µm.

Said undercoat and topcoat can independently comprise a film-forming material, chloride-vinyl acetate resin, and a coloring agent, and optional one or more of an adjusting agent and conventional auxiliary agent such as leveling agent and anti-settling agent, etc.. In the undercoat or the topcoat, relative to 100 parts by weight of the film-forming material, the content of said chloride-vinyl acetate resin can be 2 to 50 parts by weight, preferably 5 to 40 parts by weight, and more preferably 10 to 30 parts by weight; the content of said coloring agent can be 3 to 80 parts by weight, preferably 10 to 70 parts by weight, and more preferably 20 to 60 parts by weight; the content of said adjusting agent can be 0 to 20 parts by weight, preferably 2 to 15 parts by weight, and more preferably 5 to 12 parts by weight; and the content of said auxiliary agent can be 0 to 20 parts by weight, preferably 2 to 15 parts by weight, and more preferably 5 to 12 parts by weight.

Said intermediate coat can comprise film-forming material, and optional one or more of a coloring agent, an adjusting agent, and conventional auxiliary agent such as leveling agent and anti-settling agent, etc. In the intermediate coat, relative to 100 parts by weight of the film-forming material, the content of said coloring agent can be 0 to 80 parts by weight, preferably 10 to 70 parts by weight, and more preferably 20 to 60 parts by weight; the content of said adjusting agent can be 0 to 20 parts by weight, preferably 2 to 15 parts by weight, and more preferably 5 to 12 parts by weight; and the content of said auxiliary agent can be 0 to 20 parts by weight, preferably 2 to 15 parts by weight, and more preferably 5 to 12 parts by weight.

Said film-forming material can be any conventional film-forming material used in the prior art coated products; for example, the film-forming material contained in the undercoat, the intermediate coat, and the topcoat may be each independently one or more selected from a thermoplastic acrylate resin, a hydroxy acrylic resin, a self-curing alkyd resin, and an aldehyde ketone resin, and among them the thermoplastic acrylate resin is preferred. Said thermoplastic acrylate resin has been well known to those skilled in the art, and is commercially available or prepared through the copolymerization of acrylate, methacrylate, and other olefin monomers by a known method. For example, said thermoplastic acrylate resin can include, but not limited to ICI2103, ICI2106, Rohm&Haas A-11, Rohm&Haas A-12, Rohm&Haas B60, Rohm&Haas B66, Rohm&Haas A-21, Mitsubishi BR-113, Mitsubishi BR-116, Mitsubishi MB-2952, Mitsubishi MB2660, Mitsui 101, and Mitsui 102, etc. Above trade names are well known to those skilled in the art.

The chloride-vinyl acetate resin contained in said undercoat and said topcoat can be each independently one or more selected from vinyl chloride-vinyl acetate, vinyl chloride-vinyl acetate-hydroxy acrylate, vinyl chloride-vinyl acetate-maleate, and vinyl chloride-vinyl acetate-vinyl alcohol ester. Based on its total weight, the chloride-vinyl acetate resin contains 50 to 95 wt%, preferably 70 to 90 wt% of vinyl chloride; 5 to 40 wt%, preferably 8 to 25 wt% of vinyl acetate; 0 to 20 wt%, preferably 0.5 to 10 wt% of hydroxy acrylate; 0 to 20 wt%, preferably 0.5 to 10 wt% of vinyl alcohol; and 0 to 10 wt%, preferably 0.5 to 5 wt% of maleic acid. The chloride-vinyl acetate resin has a number-average molecular weight of 10000 to 50000, preferably 13000 to 42000. Said chloride-vinyl acetate resin is commercially available, such as E15/45M from Eastman, VINNOL LL4320 from WACKER (Germany), UCAR VAGH, UCAR VAGK and VMCH from UCAR (USA), T-33 from BSK (Canada), and SOBIN A from SOBIN (Japan), etc.

Said chloride-vinyl acetate resin is insoluble in alcohol solvents, for example, vinyl chloride-vinyl acetate is insoluble in alcohol, and therefore has high alcohol resistance.. Since said topcoat and undercoat contain the chloride-vinyl acetate resin, they have alcohol resistance, and therefore will not be affected when the coating is scrubbed with alcohol or alcoholic solution. Since the intermediate coat does not contain the chloride-vinyl acetate resin, it ihas no alcohol resistance, and therefore, the residual intermediate coat on the backlight part can be scrubbed off easily with alcohol or alcoholic solution.

Said coloring agent can be any conventional coloring agent used in the prior art coated products, for example, the coloring agent contained in said undercoat, intermediate coat, and topcoat can be each independently one or more selected from color slurry, pearlescence, fluorescent powder, dye, organic pigment, and inorganic pigment. Said organic pigment can include, but not limited to carbon black and titanium white. Said organic pigment can include, but not limited to azoic triaryl methane, anthraquinone, phthalocyanine, thioindigo, isoindazole ketone, quinaldine ketone, triphenyl diazine, and methylenimine groups, etc. Said coloring agent is commercially available, for example, the white color slurry can be Dema TC21 from Shibis or oily color slurry 844-0061 from DEGUSSA.

The coloring agent contained in the undercoat can be selected with reference to the expected backlight color; and the coloring agent contained in the topcoat can be determined with reference to the appearance color of said multi-layer coated product as required, as long as the undercoat and the topcoat are in a different color. Said intermediate coat contains or doesn't contain the coloring agent; if said intermediate coat contains color blending agent, the color blending agent can be any one or a mixture of above coloring agents. Preferably, said intermediate coat is in black color, because a black intermediate coat has higher light absorbing capability and can absorb more laser radiation, to facilitate the black intermediate coat and the topcoat to burn quickly and form clear engraved pattern. More preferably, said intermediate coat contains carbon black to form a black intermediate coat. Since carbon black is easy to burn at heating, the intermediate coat containing carbon black can be easily removed by the laser engraving.

Said adjusting agent can be any conventional adjusting agent in the prior art coated products, for example, the adjusting agent contained in said undercoat, intermediate coat, and topcoat can be independently selected from cellulose acetate butyrate (CAB) and rottweil powder. Said adjusting agent is used to adjust the arrangement of said coloring agent and surface properties of the coat layers. Said intermediate coat preferably contains CAB as the adjusting agent, because CAB can further reduce the alcohol resistance of the intermediate coat to easily remove the residual intermediate coat with alcohol or alcoholic solution.

The type and amount of said leveling agent is well known to those skilled in the art; for example, the leveling agent contained in said undercoat, intermediate coat, and topcoat can be each independently one or more selected from EFKA3883, EFKA3886, EFKA3600, EFKA3777, BYK366, BYK333, BYK307, and DEGO410. Among them, EFKA series are the products of EFKA (Netherland), BYK series are products of BYK Company, and DEGO series are products of DEGO (Germany); and above trade names are well known to those skilled in the art.

Said anti-settling agent is used to form powerful network structure in the resin composition to afford excellent thixotropic property to the system, so as to effectively prevent settlement and agglomeration of the color filler in the coating. The type and volume of said anti-settling agent are known to those skilled in the art; for example, Agent 201P or 229 from Taiwan Deuchem, DS6500/6800-20X or DS5000-10X from TAVY (USA), and 6900-20X or 4200-10 from Kusumoto Chemicals, Ltd. (Japan) can be used; above trade names are well known to those skilled in the art.

The multi-layer coated product provided by the present invention can be used as a component for any appliance that requires backlight pattern, and is especially suitable for keyboards or keys of electronic products. As required, the intermediate coat and topcoat in the backlight pattern part can be removed to expose the undercoat and exhibit the backlight pattern. Said substrate can be any conventional substrate applicable to components that require backlight pattern, and plastic material is preferred.

The preparation method for multi-layer coated product provided by the present invention includes the step of forming an undercoat and a topcoat which have alcohol resistance and are in a different color from each other on a substrate in sequence, wherein it further includes the step of forming an intermediate coat having no alcohol resistance between the undercoat and the topcoat.

Wherein, said undercoat, topcoat, and intermediate coat can be formed by any conventional coating preparation method, respectively. For example, the coating compostion can be mixed with a diluting agent, and the mixture is coated on the substrate and then dried. The coating composition can be mixed with the diluting agent at a weight ratio of 1: 0.5-2. Said drying method can be any prior art method, preferably drying for 5-15min. at 50-60°C. Said diluting agent can be any conventional diluting agent in the field, such as one or more of toluene, ethyl acetate, butyl acetate, isobutyl acetate, propyl acetate, ethanol, normal butyl alcohol, cyclohexanone, dimethylbenzene, methylisobutyl ketone, acetone, butanone, ethylene glycol monobutyl ether, and propylene glycol monobutyl ether.

Said undercoat can be formed with a prime coating composition; said topcoat can be formed with a finish coating composition; and said intermediate coat can be formed with an intermediate coating composition. The prime coating composition, finish coating composition, and intermediate coating composition each have the same components as the undercoat, topcoat, and intermediate coat, respectively, with the only difference that the coating compositions further contain a diluting agent. Wherein, the type and amount of said diluting agent are known to those skilled in the art. Relative to 100 parts by weight of the film-forming material, the amount of said diluting solvent is preferably 5 to 150 parts by weight, and more preferably 10 to 120 parts by weight.

Since the prime coating composition and the finish coating composition contain chloride-vinyl acetate resin having the alcohol resistance, the diluting agent in them can not be alcohol solely. In said prime coating composition and finish coating composition, said diluting agent can be one or more of toluene, ethyl acetate, butyl acetate, isobutyl acetate, propyl acetate, cyclohexanone, dimethylbenzene, methylisobutyl ketone, acetone, butanone, ethylene glycol monobutyl ether, and propylene glycol monobutyl ether, or a mixture of ethanol and/or normal butyl alcohol with one or more of the above diluting agents. In said intermediate coating composition, said diluting agent can be one or more of toluene, ethyl acetate, butyl acetate, isobutyl acetate, propyl acetate, ethanol, normal butyl alcohol, cyclohexanone, dimethylbenzene, methylisobutyl ketone, acetone, butanone, ethylene glycol monobutyl ether, and propylene glycol monobutyl ether.

Above coating compositions can be prepared with the preparation method for conventional coating compositions, for example, the components of above coating layers, such as film-forming material and optional chloride-vinyl acetate resin, coloring agent, adjusting agent, auxiliary agent, and diluting solvent, can be mixed homogeneously.

Hereunder the present invention will be described in more detail in the examples.

### Examples 1 to 5

The examples 1 to 5 are provided to prepare the coating compositions that form the coating layers.

The components shown in Table 1 were mixed homogeneously, the mixture was filtered to obtain a slurry, and then the slag was removed therefrom, to obtain the coating compositions A1, A2, A3, B1, and B2. The amount of the components in Table 1 was denoted in parts by weight.

**Table 1**

| Component | | Example 1 | Example 2 | Example 3 | Example 4 | Example 5 |
|---|---|---|---|---|---|---|
| | | A1 | A2 | A3 | B1 | B2 |
| Film-forming material | Type | Thermoplastic acrylic resin (Mitsubishi 2952) | Thermoplastic acrylic resin (Mitsubishi 2952) | Thermoplastic acrylic resin (Mitsubishi 2952) | Thermoplastic acrylic resin (Mitsubishi BR113) | Thermoplastic acrylic resin (Mitsubishi BR113) |
| | amount | 100 | 100 | 100 | 100 | 100 |
| Chloride-vinyl acetate resin | Type | Vinyl chloride-vinyl acetate-maleate (VMCH from UCAR) | Vinyl chloride-vinyl acetate (SOBIN C from SOBIN (Japan)) | Vinyl chloride-vinyl acetate-dicarbonate (LL4320 from WACKER) | - | - |
| | amount | 25 | 30 | 15 | 0 | 0 |
| Coloring agent | Type | White color slurry (Dema TC25 from Shibis) | Red color slurry (Dema TC29 from Shibis) | Green color slurry (Dema TC24 from Shibis) | Black color slurry (Dema TC21 from Shibis) | Black color slurry (Dema TC21 from Shibis) |
| | amount | 60 | 40 | 50 | 50 | 50 |
| Adjusting agent | Type | CAB resin (Eastman CAB381-20BP) | - | CAB resin (Eastman CAB381-20BP) | CAB resin (Eastman CAB381-0.5) | CAB resin (Eastman CAB381-0.5) |
| | amount | 10 | 0 | 8 | 10 | 9 |
| Anti-settling agent | Type | - | 201P from Taiwan Deuchem | 201P from Taiwan Deuchem | 201P from Taiwan Deuchem | 201P from Taiwan Deuchem |
| | amount | 0 | 3 | 3 | 3 | 3 |
| Leveling agent | Type | EFKA3883 | EFKA3883 | - | - | EFKA3883 |
| | Volume | 2 | 2 | 0 | 0 | 2 |
| Diluting agent | Type | Ethyl acetate and acetone at a weight ratio of 1: 2 | Ethyl acetate and toluene at a weight ratio of 1: 2 | Ethyl acetate and acetone at 1: 2 weight ratio | Ethyl acetate and alcohol at 1: 2 weight ratio | Ethyl acetate and normal butyl alcohol at 1: 2 weight ratio |
| | amount | 120 | 100 | 100 | 120 | 100 |

### Example 6

The example 6 is provided to describe the multi-layer coated product and the preparation method thereof according to the present invention.

Te coating composition A1 obtained in ethe example 1 was mixed with ethyl acetate in a weight ratio of 1: 0.8, and then the mixture was coated on a transparent thermoplastic keyboard, and baked for 10min. at 60°C to form the undercoat. Next, with the same method, the intermediate coat and topcoat were formed in sequence with the coating composition B1 obtained in example 4 and the coating composition A2 obtained in example 2, to obtain the multi-layer coated product D1.

### Examples 7 to 11

The examples 7 to 11 are provided to describe the multi-layer coated product and the preparation method thereof according to the present invention.

With the method used in example 6, the undercoat, intermediate coat and topcoat were formed on a transparent thermoplastic keyboard in sequence, to obtain the multi-layer coated products D2 to D6. The coating compositions used to form the undercoat, intermediate coat and topcoat were shown in Table 2 below.

### Comparative examples 1 to 3

The comparative examples 1-3 are provided to describe the multi-layer coated products of the prior art.

With the method used in example 6, the undercoat, and topcoat were formed on a transparent thermoplastic keyboard in sequence, to obtain the multi-layer coated products CD1, CD2, and CD3. The coating compositions used to form the undercoat and topcoat were shown in Table 2 below.

### Examples 12 to 17

The examples 12-17 are provided to describe the influence of the multi-layer coated products D1 to D6 prepared in examples 6-11 on the laser engraving process.

A letter "A" was engraved on the multi-layer coated products D1 to D6 prepared in examples 6 to 11 with a laser engraving machine. The laser engraving process included a pre-commissioning procedure and a post-engraving alcohol scrubbing procedure. The pre-commissioning procedure shall be carried out appropriately to ensure the engraved pattern exhibits the undercoat color, avoid residual intermediate coat or topcoat as far as possible, and prevent laser penetration into the undercoat. The post-engraving alcohol scrubbing procedure shall be carried out appropriately to ensure the dust produced in laser engraving is removed and the residual intermediate coat or topcoat is scrubbed off completely, so that the undercoat is exposed. The time for the pre-commissioning procedure, and the time for the post-engraving alcohol scrubbing procedure were recorded, and the sum of them, i.e., the total time, was calculated. The result was shown in Table 2.

### Comparative examples 4 to 6

The comparative examples 4 to 6 are provided to describe the influence of the multi-layer coated products CD1, CD2 and CD3 prepared in the comparative examples 1 to 3 on the laser engraving process.

A letter "A" was engraved on the multi-layer coated products CD1, CD2 and CD3 prepared in the comparative examples 1-3 with the method used in examples 12-17. The time for the pre-commissioning procedure, the time for the post-engraving alcohol scrubbing procedure, and the total time were recorded. The result was shown in Table 2.

**Table 2**

| Example No. | Multi-layer Coated Product No. | Coating Composition | Time (min.) for the Pre-Commissioning Procedure | Time (min.) for the Alcohol Scrubbing Procedure | Total Time (min.) |
|---|---|---|---|---|---|
| Example 12 | D1 | A1+B1+A2 | 2 | 0.5 | 2.5 |
| Example 13 | D2 | A1+B2+A2 | 2 | 0.5 | 2.5 |
| Comparative Example 4 | CD1 | A1+A2 | 8 | 5 | 13 |
| Example 14 | D3 | A1+B1+A3 | 1.5 | 0.5 | 2 |
| Example 15 | D4 | A1+B2+A3 | 2 | 0.5 | 2.5 |
| Comparative Example 5 | CD2 | A1+A3 | 10 | 6 | 16 |
| Example 16 | D5 | A2+B1+A3 | 2 | 0.5 | 2.5 |
| Example 17 | D6 | A2+B2+A3 | 1.5 | 0.5 | 2 |
| Comparative Example 6 | CD3 | A2+A3 | 9 | 8 | 17 |

It could be seen from the result in Table 2 that compared to the multi-layer coated products CD1, CD2 and CD3 obtained in the comparative examples 1-3, the multi-layer coated products D1 to D6 obtained in examples 6 to 11 of the present invention requires much less time for the pre-commissioning procedure and alcohol scrubbing procedure during the laser engraving process, which indicates that the production efficiency of the multi-layer coated product according to the present invention is prominently increased.

## Claims

1. A multi-layer coated product, comprising:
a substrate, and a multi-layer coating including an undercoat and a topcoat which are formed on the substrate in sequence, have alcohol resistance, and are in a different color from each other,
wherein the multi-layer coating further includes an intermediate coat having no alcohol resistance between the undercoat and the topcoat,
wherein the undercoat and the topcoat independently comprise a film-forming material, a chloride-vinyl acetate resin and a coloring material, and
wherein the intermediate coat comprises a film-forming material.

2. The product according to claim 1, wherein the undercoat, the topcoat, and the intermediate coat each independently have a thickness of 3 to 15 µm.

3. The product according to claim 1 or 2, wherein the undercoat and the topcoat each independently contain
100 parts by weight of a film-forming material,
2 to 50 parts by weight of chloride-vinyl acetate resin,
3 to 80 parts by weight of a coloring agent,
0 to 20 parts by weight of an adjusting agent and
0 to 20 parts by weight of an auxiliary agent;
and the intermediate coat contains
100 parts by weight of a film-forming material,
0 to 80 parts by weight of a coloring agent,
0 to 20 parts by weight of an adjusting agent and
0 to 20 parts by weight of an auxiliary agent.

4. The product according to any one of claims 1-3, wherein the film-forming material contained in the undercoat, the intermediate coat, and the topcoat is each independently one or more selected from a thermoplastic acrylate resin, a hydroxy acrylic resin, a self-curing alkyd resin, and an aldehyde ketone resin.

5. The product according to any one of claim 1-3, wherein
the chloride-vinyl acetate resin contained in the undercoat and the topcoat is each independently one or more selected from vinyl chloride-vinyl acetate, vinyl chloride-vinyl acetate-hydroxy acrylate, vinyl chloride-vinyl acetate-maleate, and vinyl chloride-vinyl acetate-vinyl alcohol ester; based on its total weight,
the chloride-vinyl acetate resin contains
50 to 95 wt% of vinyl chloride,
5 to 40 wt% of vinyl acetate,
0 to 20 wt% of hydroxy acrylate,
0 to 20 wt% of vinyl alcohol, and
0 to 10 wt% of maleic acid; and
the chloride-vinyl acetate resin has a number-average molecular weight of 10000 to 50000.

6. The product according to any one of claims 1-3, wherein the coloring agent contained in the undercoat, the intermediate coat, and the topcoat is each independently one or more selected from color slurry, pearlescence, fluorescent powder, dye, organic pigment, and inorganic pigment.

7. The product according to claim 6, wherein the coloring agent contained in the intermediate coat is carbon black which is a kind of the organic pigment.

8. The product according to any one of claims 1-3, wherein the adjusting agent contained in the undercoat, the intermediate coat, and the topcoat is each independently selected from cellulose acetate butyrate and rottweil powder; and the auxiliary agent contained in the undercoat, the intermediate coat, and the topcoat is each independently selected from anti-settling agent and leveling agent.

9. A method for preparing a multi-layer coated product, including the steps of
forming an undercoat and a topcoat which have alcohol resistance and are in a different color from each other on a substrate in sequence, and
forming an intermediate coat having no alcohol resistance between the undercoat and the topcoat,
wherein the undercoat and the topcoat independently comprise a film-forming material, a chloride-vinyl acetate resin and a coloring material, and
wherein the intermediate coat comprises a film-forming material.

10. The method according to claim 9, wherein the undercoat is formed from a prime coating composition, the topcoat is formed from a finish coating composition, and the intermediate coat is formed from a intermediate coating composition;
the prime coating composition and the finish coating composition each independently contain
100 parts by weight of a film- forming material,
2 to 50 parts by weight of chloride-vinyl acetate resin,
3 to 80 parts by weight of a coloring agent,
5 to 150 parts by weight of a diluting agent,
0 to 20 parts by weight of an adjusting agent and
0 to 20 parts by weight of an auxiliary agent; and
the intermediate coating composition contains
100 parts by weight of a film-forming material,
5 to 150 parts by weight of a diluting agent,
0 to 80 parts by weight of a coloring agent,
0 to 20 parts by weight of an adjusting agent and
0 to 20 parts by weight of an auxiliary agent.

11. The method according to claim 10, wherein the film-forming material contained in the prime coating composition, the intermediate coating composition, and the finish coating composition is each independently one or more selected from a thermoplastic acrylate resin, a hydroxy acrylic resin, a self-curing alkyd resin, and an aldehyde ketone resin.

12. The method according to claim 10, wherein the chloride-vinyl acetate resin contained in the prime coating composition and the finish coating composition is each independently one or more selected from vinyl chloride-vinyl acetate, vinyl chloride-vinyl acetate-hydroxy acrylate, vinyl chloride-vinyl acetate-maleate, and vinyl chloride-vinyl acetate-vinyl alcohol ester; based on its total weight,
the chloride- vinyl acetate resin contains
50 to 95 wt% of vinyl chloride,
5 to 40 wt% of vinyl acetate,
0 to 20 wt% of hydroxy acrylate,
0 to 20 wt% of vinyl alcohol, and
0 to 10 wt% of maleic acid; and
the chloride-vinyl acetate resin has a number-average molecular weight of 10000 to 50000.

## Patentansprüche

1. Mehrschichtig beschichtetes Produkt, umfassend:
ein Substrat und eine mehrschichtige Beschichtung, die eine Unterzugsschicht und eine Überzugsschicht umfasst, die auf dem Substrat sequenziell gebildet sind, Alkoholbeständigkeit aufweisen und voneinander verschiedene Farben besitzen,
worin die mehrschichtige Beschichtung ferner eine Zwischenbeschichtung, die keine Alkoholbeständigkeit aufweist, zwischen der Unterzugsbeschichtung und der Überzugsbeschichtung umfasst,
worin die Unterzugsbeschichtung und die Überzugsbeschichtung unabhängig voneinander ein filmbildendes Material, ein Chlorid-Vinylacetatharz und ein färbendes Material umfassen und
worin die Zwischenbeschichtung ein filmbildendes Material umfasst.

2. Produkt gemäß Anspruch 1, worin die Unterzugsschicht, die Überzugsschicht und die Zwischenschicht jeweils unabhängig eine Dicke von 3 bis 15 µm aufweisen.

3. Produkt gemäß Anspruch 1 oder 2, worin die Unterzugsschicht und die Überzugsschicht jeweils unabhängig voneinander 100 Gew.-Teile eines filmbildenden Materials,
2 bis 50 Gew.-Teile Chlorid-Vinylacetatharz,
3 bis 80 Gew.-Teile eines Färbemittels,
0 bis 20 Gew.-Teile eines Einstellmittels und
0 bis 20 Gew.-Teile eines Hilfsstoffs enthalten;
und die Zwischenschicht
100 Gew.-Teile eines filmbildenden Materials,
0 bis 80 Gew.-Teile eines Färbemittels,
0 bis 20 Gew.-Teile eines Einstellmittels und
0 bis 20 Gew.-Teile eines Hilfsstoffs
enthält.

4. Produkt gemäß irgendeinem der Ansprüche 1 bis 3, worin das filmbildende Material, das in der Unterzugsschicht, der Zwischenschicht und der Überzugsschicht enthalten ist, jeweils unabhängig voneinander eines oder mehrere ist/sind, ausgewählt aus thermoplastischem Acrylatharz, einem Hydroxy-Acrylharz, einem selbsthärtenden Alkydharz und einem Aldehyd-Ketonharz.

5. Produkt gemäß irgendeinem der Ansprüche 1 bis 3, worin
das Chlorid-Vinylacetatharz, das in der Unterzugsschicht und der Überzugsschicht enthalten ist, jeweils unabhängig voneinander eines oder mehrere ist/sind, ausgewählt aus Vinylchlorid-Vinylacetat, Vinylchlorid-Vinylacetat-Hydroxyacrylat, Vinylchlorid-Vinylacetat-Maleat und Vinylchlorid-Vinylacetat-Vinylalkoholester; und, bezogen auf sein Gesamtgewicht,
das Chlorid-Vinylacetatharz
50 bis 95 Gew.% Vinylchlorid,
5 bis 40 Gew.% Vinylacetat,
0 bis 20 Gew.% Hydroxyacrylat,
0 bis 20 Gew.% Vinylalkohol und
0 bis 10 Gew.% Maleinsäure enthält; und
das Chlorid-Vinylacetatharz ein zahlengemitteltes Molekulargewicht von 10.000 bis 50.000 aufweist.

6. Produkt gemäß irgendeinem der Ansprüche 1 bis 3, worin das Färbemittel, das in der Unterzugsschicht, der Zwischenschicht und der Überzugsschicht enthalten ist, jeweils unabhängig voneinander eines oder mehrere ist/sind, ausgewählt aus einer Farbaufschlämmung, Perlenglanz, fluoreszierendem Pulver, Farbstoff, organischem Pigment und anorganischem Pigment.

7. Produkt gemäß Anspruch 6, worin das Färbemittel, das in der Zwischenschicht enthalten ist, Ruß ist, welche eine Art des organischen Pigments ist.

8. Produkt gemäß irgendeinem der Ansprüche 1 bis 3, worin das Einstellmittel, das in der Unterzugsschicht, der Zwischenschicht und der Überzugsschicht enthalten ist, jeweils unabhängig voneinander ausgewählt ist aus Zelluloseacetatbutyrat und Rottweil-Pulver; und der Hilfsstoff, der in der Unterzugsschicht, der Zwischenschicht und der Überzugsschicht enthalten ist, jeweils unabhängig ausgewählt ist aus Anti-Setzmitteln und Nivelliermitteln.

9. Verfahren zum Herstellen eines mehrschichtig beschichteten Produkts, umfassend die Schritte
Bilden einer Unterzugsschicht und einer Überzugsschicht, die Alkoholbeständigkeit aufweisen und voneinander unterschiedliche Farben besitzen, nacheinander auf einem Substrat, und
Bilden einer Zwischenschicht, die keine Alkoholbeständigkeit aufweist, zwischen der Unterzugsschicht und der Überzugsschicht,
worin die Unterzugsschicht und die Überzugsschicht unabhängig voneinander ein filmbildendes Material, ein Chlorid-Vinylacetatharz und ein färbendes Material umfassen, und
worin die Zwischenschicht ein filmbildendes Material umfasst.

10. Verfahren gemäß Anspruch 9, worin die Unterzugsschicht aus einer Grundierungs-Beschichtungszusammensetzung gebildet ist, die Überzugsschicht aus einer Finish-Beschichtungszusammensetzung gebildet ist und die Zwischenschicht aus einer
Zwischenbeschichtungszusammensetzung gebildet ist; worin die Grundierungs-Beschichtungszusammensetzung und die Finish-Beschichtungszusammensetzung jeweils unabhängig voneinander enthalten
100 Gew.-Teile eines filmbildenden Materials,
2 bis 50 Gew.-Teile Chlorid-Vinylacetatharz,
3 bis 80 Gew.-Teile eines Färbemittels,
5 bis 150 Gew.-Teile eines Verdünnungsmittels,
0 bis 20 Gew.-Teile eines Einstellmittels und
0 bis 20 Gew.-Teile eines Hilfsstoffs; und
die Zwischenbeschichtungszusammensetzung enthält
100 Gew.-Teile eines filmbildenden Materials
5 bis 150 Gew.-Teile eines Verdünnungsmittels,
0 bis 80 Gew.-Teile eines Färbemittels,
0 bis 20 Gew.-Teile eines Einstellmittels, und
0 bis 20 Gew.-Teile eines Hilfsstoffs.

11. Verfahren gemäß Anspruch 10, worin das filmbildende Material, das in der Grundierungs-Beschichtungszusammensetzung, der Zwischenbeschichtungszusammensetzung und der Finish-Beschichtungszusammensetzung enthalten ist, jeweils unabhängig eines oder mehrere ist/sind, ausgewählt aus einem thermoplastischen Acrylatharz, einem Hydroxy-Acrylharz, einem selbsthärtenden Alkydharz und einem Aldehyd-Ketonharz.

12. Verfahren gemäß Anspruch 10, worin das Chlorid-Vinylacetatharz, das in der Grundierungs-Beschichtungszusammensetzung und der Finish-Beschichtungszusammensetzung enthalten ist, jeweils unabhängig eines oder mehrere ist/sind, ausgewählt aus Vinylchlorid-Vinylacetat, Vinylchlorid-Vinylacetat-Hydroxyacrylat, Vinylchlorid-Vinylacetat-Maleat und Vinylchlorid-Vinylacetat-Vinylalkoholester; und, bezogen auf sein Gesamtgewicht, das Chlorid-Vinylacetatharz 50 bis 95 Gew.% Vinylchlorid,
5 bis 40 Gew.% Vinylacetat,
0 bis 20 Gew.% Hydroxyacrylat,
0 bis 20 Gew.% Vinylalkohol und
0 bis 10 Gew.% Maleinsäure
enthält; und
das Chlorid-Vinylacetatharz ein zahlengemitteltes Molekulargewicht von 10.000 bis 50.000 aufweist.

## Revendications

1. Produit revêtu multicouche, comprenant :
un substrat, et un revêtement multicouche comportant une sous-couche et une couche de finition qui sont formées séquentiellement sur le substrat, ont une résistance aux alcools, et ont des couleurs différentes,
où le revêtement multicouche comporte en outre une couche intermédiaire n'ayant pas de résistance aux alcools entre la sous-couche et la couche de finition,
où la sous-couche et la couche de finition comprennent indépendamment un matériau filmogène, une résine chlorure-acétate de vinyle et un matériau colorant, et
où la couche intermédiaire comprend un matériau filmogène.

2. Produit selon la revendication 1, dans lequel la sous-couche, la couche de finition, et la couche intermédiaire ont chacune indépendamment une épaisseur allant de 3 à 15 µm.

3. Produit selon la revendication 1 ou 2, dans lequel la sous-couche et la couche de finition contiennent chacune indépendamment
100 parties en poids d'un matériau filmogène,
2 à 50 parties en poids de résine chlorure-acétate de vinyle,
3 à 80 parties en poids d'un agent colorant,
0 à 20 parties en poids d'un agent de régulation et
0 à 20 parties en poids d'un agent auxiliaire ;
et la couche intermédiaire contient
100 parties en poids d'un matériau filmogène,
0 à 80 parties en poids d'un agent colorant,
0 à 20 parties en poids d'un agent de régulation et
0 à 20 parties en poids d'un agent auxiliaire.

4. Produit selon l'une quelconque des revendications 1-3, dans lequel les matériaux filmogènes contenus dans la sous-couche, la couche intermédiaire, et la couche de finition sont chacun indépendamment un ou plusieurs éléments choisis parmi une résine acrylique thermoplastique, une résine hydroxyacrylique, une résine alkyde auto-polymérisable, et une résine de cétone aldéhyde.

5. Produit selon l'une quelconque des revendications 1-3, dans lequel
les résines chlorure-acétate de vinyle contenues dans la sous-couche et la couche de finition sont chacune indépendamment un ou plusieurs éléments choisis parmi le chlorure de vinyle-acétate de vinyle, le chlorure de vinyle-acétate de vinyle-hydroxy acrylate, le chlorure de vinyle-acétate de vinyle-maléate, et le chlorure de vinyle-acétate de vinyle-ester d'alcool de vinyle ; par rapport à son poids total,
la résine chlorure-acétate de vinyle contient
50 à 95% en poids de chlorure de vinyle,
5 à 40% en poids d'acétate de vinyle,
0 à 20% en poids d'hydroxy acrylate,
0 à 20% en poids d'alcool de vinyle, et
0 à 10% en poids d'acide maléique ; et
la résine chlorure-acétate de vinyle a une masse moléculaire moyenne en nombre allant de 10000 à 50000.

6. Produit selon l'une quelconque des revendications 1-3, dans lequel les agents colorants contenus dans la sous-couche, la couche intermédiaire, et la couche de finition sont chacun indépendamment un ou plusieurs éléments choisis parmi une suspension de couleur, une essence d'orient, une poudre fluorescente, un colorant, un pigment organique, et un pigment inorganique.

7. Produit selon la revendication 6, dans lequel l'agent colorant contenu dans la couche intermédiaire est du noir de carbone qui est un type du pigment organique.

8. Produit selon l'une quelconque des revendications 1-3, dans lequel les agents de régulation contenus dans la sous-couche, la couche intermédiaire, et la couche de finition sont chacun indépendamment choisis d'une poudre de Rottweil et d'acétate butyrate de cellulose ; et les agents auxiliaires contenus dans la sous-couche, la couche intermédiaire, et la couche de finition sont chacun indépendamment choisis parmi un agent stabilisateur et un agent d'unisson.

9. Procédé destiné à préparer un produit revêtu multicouche, comportant les étapes consistant
à former séquentiellement une sous-couche et une couche de finition qui ont une résistance aux alcools et ont des couleurs différentes sur un substrat, et
à former une couche intermédiaire n'ayant pas de résistance aux alcools entre la sous-couche et la couche de finition,
où la sous-couche et la couche de finition comprennent indépendamment un matériau filmogène, une résine chlorure-acétate de vinyle et un matériau colorant, et
où la couche intermédiaire comprend un matériau filmogène.

10. Procédé selon la revendication 9, dans lequel la sous-couche est formée d'une composition de revêtement primaire, la couche de finition est formée d'une composition de revêtement de finition, et la couche intermédiaire est formée d'une composition de revêtement intermédiaire ;
la composition de revêtement primaire et la composition de revêtement de finition contiennent chacune indépendamment
100 parties en poids d'un matériau filmogène,
2 à 50 parties en poids de résine chlorure-acétate de vinyle,
3 à 80 parties en poids d'un agent colorant,
5 à 150 parties en poids d'un agent de dilution,
0 à 20 parties en poids d'un agent de régulation et
0 à 20 parties en poids d'un agent auxiliaire ; et
la composition de revêtement intermédiaire contient
100 parties en poids d'un matériau filmogène,
5 à 150 parties en poids d'un agent de dilution,
0 à 80 parties en poids d'un agent colorant,
0 à 20 parties en poids d'un agent de régulation et
0 à 20 parties en poids d'un agent auxiliaire.

11. Procédé selon la revendication 10, dans lequel les matériaux filmogènes contenus dans la composition de revêtement primaire, la composition de revêtement intermédiaire, et la composition de revêtement de finition sont chacun indépendamment un ou plusieurs éléments choisis parmi une résine acrylique thermoplastique, une résine hydroxyacrylique, une résine alkyde auto-polymérisable, et une résine de cétone aldéhyde.

12. Procédé selon la revendication 10, dans lequel les résines chlorure-acétate de vinyle contenues dans la composition de revêtement primaire et la composition de revêtement de finition sont chacune indépendamment un ou plusieurs éléments choisis parmi le chlorure de vinyle-acétate de vinyle, le chlorure de vinyle-acétate de vinyle-hydroxy acrylate, le chlorure de vinyle-acétate de vinyle-maléate, et le chlorure de vinyle-acétate de vinyle-ester d'alcool de vinyle ; par rapport à son poids total,
la résine chlorure-acétate de vinyle contient
50 à 95% en poids de chlorure de vinyle,
5 à 40% en poids d'acétate de vinyle,
0 à 20% en poids d'hydroxy acrylate,
0 à 20% en poids d'alcool de vinyle, et
0 à 10% en poids d'acide maléique ; et
la résine chlorure-acétate de vinyle a une masse moléculaire moyenne en nombre allant de 10000 à 50000.
